

No. 696,270.

Patented Mar. 25, 1902.

K. RENDSCHMIDT.  
FLASH LIGHT CARTRIDGE.

(Application filed Jan. 16, 1902.)

(No Model.)

Fig. 1.



Fig. 2.



Witnesses:

Isabella Baldwin  
Addaude Claire Gleason

Inventor:  
Karl Rendschmidt  
by *Richard D.*  
Attorneys.

# UNITED STATES PATENT OFFICE.

KARL RENDSCHMIDT, OF BERLIN, GERMANY.

## FLASH-LIGHT CARTRIDGE.

SPECIFICATION forming part of Letters Patent No. 696,270, dated March 25, 1902.

Application filed January 16, 1902. Serial No. 90,012. (No model.)

To all whom it may concern:

Be it known that I, KARL RENDSCHMIDT, engineer, a citizen of the Kingdom of Prussia, and a resident of Berlin, Germany, (whose post-office address is Wilsnackerstrasse 19,) have invented certain new and useful Improvements in Flash - Light Cartridges, of which the following is a specification.

The present invention relates to flash-light cartridges which have been formed by compressing measured quantities of magnesium or similar powder into the form of small cakes or tablets. It is a known fact that by compressing flash-light powder into solid masses the inflammability of same is considerably reduced and that ignition only will be possible by aid of a peculiar primer. The photographer who intends to use these cartridges is therefore obliged to carry primers besides the cartridges.

The object of the present invention, of which Figure 1 of the accompanying drawings shows a perspective view, and Fig. 2 a vertical section, is a cartridge which, besides the necessary quantity of magnesium, &c., powder also contains the primer, which is easily separated from the cartridge proper and then is easily ignited by means of saltpeter paper, causing by its ignition the explosion of the cartridge.

The cartridge may have any convenient form—square, round, hexagonal, &c. A small part of it, which is separated from the rest by a groove, may be easily broken off and pulverized between the fingers, this powder serving for a primer.

In the drawings, *a* is the cartridge, which has the form of a flat round disk. A small part *b* of the same may be easily broken off, a groove *c* facilitating said operation. As it will be difficult to disintegrate the part *b* when the cartridge is heavily compressed, and as, on the other hand, it is of great importance to reduce the volume of the cartridge and render it as hard as possible I intend to form the cartridges in such a way that the cartridge proper will be highly compressed, whereas the detachable primer is of softer consistency.

For that purpose I proceed in manufacturing the cartridges in such a way that I do not distribute the flash-light powder uniformly over the whole form in which the pressing is done, but bring in the powder in such a way that a thicker layer is formed on the part corresponding to the cartridge proper and a thinner one on the part to be occupied by the primer. The disk on entering the form therefore will compress the former part stronger than the latter one.

In order to do away with the necessity of carrying saltpeter paper for igniting the primer, the whole cartridge may be wrapped in a piece of same and may be brought in this form into the market. Each cartridge then contains all that is necessary for making a flash-light exposure.

What I claim is—

1. A flash-light cartridge of compressed flash-light powder, part of which may be easily separated from the rest, said part serving after disintegration as a primer for igniting the cartridge proper.

2. A flash-light cartridge consisting of the cartridge proper and the primer, said primer being easily detached from the cartridge, said cartridge and primer forming a homogeneous mass.

3. A flash-light cartridge, comprising the cartridge proper and an easily-detachable primer, the cartridge containing the powder in highly-compressed state, whereas the powder forming the primer is less compressed.

4. Process for manufacturing flash-light cartridges consisting of a cartridge proper and an easily-detachable primer, consisting in filling the part of the form corresponding to the cartridge proper with a thicker layer of powder than the part corresponding to the primer.

In testimony whereof I affix my signature in presence of two witnesses.

KARL RENDSCHMIDT.

Witnesses:

WOLDEMAR HAUPT,  
HENRY HASPER.